

Sept. 29, 1931.

J. J. BOWDEN

1,824,865

PROCESS OF HEAT TREATING METAL

Filed Dec. 29, 1930



Fig. 2

James J. Bowden  
By Hall Brock & West

Inventor

Attorney

## UNITED STATES PATENT OFFICE

JAMES J. BOWDEN, OF WARREN, OHIO

## PROCESS OF HEAT-TREATING METAL

Application filed December 29, 1930. Serial No. 505,353.

This invention relates to a process of heat treating metals in any desired form, either as machine parts or raw or partly prepared material for the manufacture of metal products. This process is intended more especially for use in heat treating large charges where absolute evenness of treatment is not indispensable but where high grade and uniform quality is desirable. In the past the trade has been forced to tolerate a rather inferior type of heat treatment because uniformity and high quality could not be economically secured by the employment of known methods. Box annealing has been carried out by placing the charge, often several tons, in a heavy cast iron or similar heavy metallic annealing box, inserting said box into a furnace where the flames and products of combustion are brought into direct contact therewith. The construction of furnaces used in this process have not led to uniform temperatures in all parts of the charge.

The principal object of my invention is to provide a process for heat treating large charges which will result in the production of a more nearly uniformly treated and therefore superior product, a saving of fuel, a greater simplicity and nicety of temperature control and a saving in the time required to carry out the process. More limited objects of my invention are to combine the features of exclusion of air from the charge of metal to be treated with that of preventing access to such charge of the material which is employed for transmitting heat thereto, to reduce to a minimum the amount of heating material required while securing the advantage of retaining such material at a temperature not excessively lower than its normal maximum during the entire time the process is being carried out. Other and more limited objects will become apparent as the description proceeds.

In the accompanying drawings I have illustrated schematically the apparatus which I employ in carrying out my improved process. Fig. 1 is a schematic plan view of a series of vats V each of which is to be associated with some form of heating

means indicated at H. Each vat is to contain a molten material which at its melting point will have a temperature substantially lower than that to which the charge of material to be treated is desired to be brought. Such molten material may consist of any one of a large number of salts, such, for example, as sodium carbonate, sodium chloride, sodium hydroxide, sodium sulphate, in fact, the common salts or compounds of potassium, calcium, sodium, barium, bismuth and magnesium. I may also employ molten metals, such as lead, tin, zinc, copper, etc.

In its simplest aspect, as shown in Fig. 2 of the drawings, my improved method will consist in immersing the annealing box A containing the charge C of metal to be annealed in the molten liquid L, allowing it to remain there until it assumes the desired temperature, preferably substantially that of the liquid L, and then subjecting to any type of cooling desired to bring out the particular characteristic of the metal which is to be secured. The apparatus illustrated may be employed for the cooling treatment or additional apparatus may be used. The container A will preferably consist of an iron or steel receptacle.

By the use of a plurality of vats, each containing a different molten liquid, it is possible to secure a number of different temperatures by the simple expedient of removing the annealing box from one vat to the other. In this way, I am enabled to subject the charge to gradual heating and gradual cooling, to retain the same at substantially any temperature for as long as may be required, and to reduce the capacity of each vat very considerably without excessively lowering the temperature of the liquid L, which might result in the undesirable effect of freezing the liquid, by the simple expedient of immersing the annealing box in solutions of successively higher temperatures until the desired temperature is attained.

A very important feature of my invention is the sealing of the charge in the air-tight and liquid-tight annealing box A before it is immersed in the heating liquid and se-

curing the double function of excluding the charge from atmosphere and the surrounding heating medium. It is to be noted that various mixtures may be used to secure various melting temperatures of the liquid L. For example, a mixture of soda ash and sodium hydroxide or a mixture of copper and tin, lead and tin, may be employed. The proper control of the temperature is quite important since a number of metals, such as iron, steel, brass, zinc, aluminum, etc., have critical temperatures at which various metallurgical changes in structural composition occur.

15 Having thus described my invention, what I claim is:

1. The method of heat treatment which consists in enclosing the charge to be treated in an air-tight and liquid-tight container, 20 immersing said container with its contained charge in a molten heating agent and allowing it to remain so immersed until the charge assumes substantially the temperature of said molten heating agent.

25 2. The method of heat treating metal which consists in enclosing a charge of the metal to be treated in a container, submerging said container with its contained charge in a molten heating agent and allowing it 30 to remain therein until the desired metallurgical effect has been secured, said container being of such construction as to prevent the entrance thereinto of said heating agent.

35 3. The method of heat treating metal which consists in enclosing a charge of the metal to be treated in a substantially air-tight and liquid-tight container, at least 40 partially covering said container with its contained charge with a molten heating agent and allowing it to remain therein until the desired metallurgical effect has been secured.

45 In testimony whereof, I hereunto affix my signature.

JAMES J. BOWDEN.